

## UNITED STATES PATENT OFFICE.

HARRY W. CHARLTON AND RANDOLPH NORRIS SHREVE, OF NEW YORK, N. Y.,  
ASSIGNORS TO AMERICAN POTASH CORPORATION, OF NEW YORK, N. Y., A  
CORPORATION OF VIRGINIA.

## ACCELERATING AGENT IN POTASH RECOVERY.

No Drawing.

Application filed March 5, 1921. Serial No. 449,913.

*To all whom it may concern:*

Be it known that we, HARRY W. CHARLTON and RANDOLPH NORRIS SHREVE, respectively a citizen of Canada and a citizen of the 5 United States, each residing at New York, in the county of New York and State of New York, have invented certain new and useful Improvements Regarding Accelerating Agent in Potash Recovery; and we do 10 hereby declare the following to be a full, clear, and exact description of the invention, such as will enable others skilled in the art to which it appertains to make and use the same.

15 This invention relates to a method of accelerating the liberation of potassium salts during processes of digestion and thereby recovering a greater proportion of potassium in a more expeditious and less costly manner than heretofore proposed.

With these and other objects in view, the invention consists in the novel steps and combination of steps constituting the process and in the novel catalytic or accelerating 25 agent employed, all as will be more fully hereinafter disclosed and particularly pointed out in the claims.

In order that the precise invention may be more clearly understood, it is said:

30 When a mixture of greensand, lime and water are digested at elevated temperatures and under superatmospheric pressures for a suitable period, a very considerable percentage of the potassium is rendered soluble and 35 appears in the digestion liquor as potassium hydrate.

In a copending application of Charlton and Shreve on alkali metal products of even date, an invention is described in which various sodium salts react with the caustic potash formed, from the action of lime and water on greensand, and thus give caustic soda, and the corresponding potassium salt,—this action being accompanied by an 45 increase in the yield.

We have discovered that the addition of certain potassium salts speeds up the reaction as well as increases the yield in these cases.

50 According to this invention, one may take, for example, by weight, say, 85 parts of finely divided greensand, add thereto 85 parts of quick lime, or  $\text{CaO}$ , and 12 parts of potassium nitrate,  $\text{KNO}_3$ , mixed with 425

parts of water, and digest the mixture at, 55 say,  $470^{\circ}$  Fahrenheit, corresponding to a pressure of about 500 pounds, for about 40 minutes; when it will be found that about 69% of the total potassium originally present in the greensand will appear in the resulting solution in the form of potassium hydroxide. This solution may now be filtered, the filtrate evaporated, and the potassium nitrate, which was added, recovered in any suitable well known manner, as by 60 65 crystallization.

A surprising accelerating action is found to result from the addition of the potassium nitrate to the digestion mixture, in that with the said nitrate present a higher yield of 70 potassium from the greensand is obtained, than is the case when no potassium nitrate is present.

In a specific instance, it was found that only 61% of potassium present in the greensand appeared in the soluble form when no potassium nitrate was used, while more than 68% of said potassium was dissolved, under precisely the same conditions when potassium nitrate was employed. In this case, 75 80 the potassium that was dissolved out of the greensand was found to be in the form of the hydrate, practically all of the potassium nitrate added being readily recoverable.

In other words, it has been found that the 85 potassium nitrate thus employed can, after recovery, be used over again and thus made to act somewhat after the manner of a catalyst to accelerate the dissolving out of the potassium present in the greensand. 90

In another specific test, 10 parts of calcium nitrate were added to the digestion mixture when more than 72% of the potassium present in the greensand was dissolved. But in omitting said calcium nitrate under precisely the same conditions, less than 62% of the potassium present in the greensand was found in the filtrate. In still another test, using ammonium nitrate, it was found that the potassium yield was increased thereby 95 to 78%, from less than 62%. 100

Similarly the additions of other salts to the greensand, lime, water mixture before digestion accelerates the action of the lime in decomposing the greensand. For example, the addition of about 6 parts of ammonium chloride increases the amount of potassium dissolved out of the greensand 105

from less than 48% to over 67%. (In this case the digestion period was only 20 minutes.)

The explanation of the accelerating action 5 of the various salts upon the liberation of the potassium from the greensand is probably due to an increase in the amount of the calcium hydroxide or of the calcium ion in the solution, due to the action of the 10 added salt. As evidence of this probable explanation I refer to Gmelin-Kraut's Hand-

buch der anorganischen Chemie, 7th edition, volume II, part 2, pages 206, 207, 208, in which much data is collected together showing 15 the increase in amount of calcium hydroxide or calcium ions in aqueous solution in presence of various dissolved compounds, in comparison with solubility in water alone.

Among such salts which increase the solubility 20 of calcium hydroxide, are nitrates of sodium, potassium and calcium; sodium sulphate, sodium chloride, ammonium chloride, etc., etc. Data is also given in this same reference showing that while caustic 25 potash and caustic soda solutions dissolve less calcium hydroxide than pure water, yet certain salts, for example calcium nitrate, actually dissolve in caustic soda and caustic potash solutions to such an extent as to increase 30 the amount of calcium ions present, over what would be present under the same conditions without the calcium nitrate.

Although this process has been exemplified largely by its application to greensand, 35 yet it is found that it will operate on the distantly related leucite, phonolite, etc., and other potassium silicate bearing rocks, in a manner similar to that disclosed in connection with greensand.

40 In carrying out the digestion with greensand, etc., it is preferred to grind it, preferably to pass a screen of 200 mesh, as the

reaction is hastened and the yield accordingly increased.

Although the above examples have employed 45 pressures of about 500 pounds, such pressures are not at all necessary, because pressures all the way from, say 100 pounds up to over 500 pounds may be employed, provided that the time of digestion is varied accordingly. It is found, of course, that the higher the pressure the less will be the time of digestion.

It is obvious that those skilled in the art 50 may vary the details of the process without departing from the spirit of the invention, and therefore we do not wish to be limited to the above disclosures except as may be required by the claims.

We claim:

1. The process of accelerating the recovery 55 of the potassium contained in greensand, which consists in digesting said greensand with potassium nitrate, and milk of lime under a super-atmospheric pressure and at a corresponding temperature, substantially as described.

2. The process of recovering combined 60 potassium from greensand which consists in heating under superatmospheric pressure 70 said material admixed with lime, water and an accelerating agent containing potassium nitrate, substantially as described.

3. The process of accelerating the action 75 of lime and water in dissolving potassium from greensand when heated under superatmospheric conditions, which consists in adding potassium nitrate to a mixture of said lime, water and sand, substantially as described.

In testimony whereof we affix our signatures.

HARRY W. CHARLTON,  
RANDOLPH NORRIS SHREVE.